

May 25, 1948.

W. J. KRUPPA ET AL

2,442,173

PRODUCTION OF PRIMARY ULTRAMARINE

Filed July 24, 1945



INVENTORS  
WILLIAM J. KRUPPA,  
ALLING P. BEARDSLEY,  
STANLEY H. WHITING,  
BY  
Robert James Morris  
ATTORNEY

## UNITED STATES PATENT OFFICE

2,442,173

## PRODUCTION OF PRIMARY ULTRAMARINE

William J. Kruppa, Middlesex, Alling P. Beardsley, Plainfield, and Stanley H. Whiting, Martinsville, N.J., assignors to American Cyanamid Company, New York, N.Y., a corporation of Maine

Application July 24, 1945, Serial No. 606,759

5 Claims. (Cl. 106—305)

1

This invention relates to an improvement in the production of ultramarine.

Up to now the standard commercial procedure for ultramarine has involved the charging of the raw mix containing china clay, silica, soda ash, sulfur, and a carbonaceous reducing agent such as pitch or rosin, into ceramic pots or crucibles of fairly small size, which are then stacked into a single furnace which normally contains more than 1,000 crucibles. The furnace is then fired up to a certain temperature, held there for a sufficient time to produce primary ultramarine from the raw mix, which is a product that is weak and dull in shade, followed by a very slow cooling time, which takes a couple of weeks, during which oxygen passes through the walls of the crucibles, which are of carefully controlled porosity, and oxidizes the primary ultramarine to the stronger and brighter secondary ultramarine which is the pigment of commerce. This operation removes about one-seventh to one-eighth of the combined sodium in the primary ultramarine.

In the copending applications of Beardsley and Whiting, Serial No. 606,887, filed July 24, 1945, and Serial No. 606,888, filed July 24, 1945, there is described and claimed an improved two-step process in which the production of primary ultramarine is effected in substantially impervious ceramic containers, such as crucibles, and then the oxidation step is effected in the same or a different furnace under conditions which permit regulated control of the contact of the oxidizing gases with the primary ultramarine. In one of said applications there is also described and claimed the use of sulfur dioxide as an oxidizing agent in the second step of the process.

The two processes have the first or primary ultramarine firing in common. Various reactions appear to take place in the production of the primary ultramarine and these reactions require different times and different temperatures. In the process as ordinarily used there is little control possible. The crucibles are stacked in the furnace and the furnace is then fired. The crucibles nearest the fire heat up most rapidly and reach top temperature first. It is therefore necessary to over-heat the crucibles nearest the fire in order to bring the more distant ones to a sufficiently high temperature, or else a compromise must be struck in which some of the crucibles near the fire are somewhat over-heated, the crucibles in the middle of the furnace are heated to the right temperature, and the more distant crucibles are somewhat underheated.

It has been proposed, and in some cases put

into practice, to use multiple hearths so that the distances that the heating gases have to pass is less. This introduces a serious complication as it is extremely difficult, in fact almost impossible, to control the individual fires perfectly evenly.

The procedure used in the past not only results in uneven temperatures in the different crucibles but the rate at which the temperature is raised cannot be accurately controlled. The whole operation is a necessary, although undesirable, compromise with preferred operating conditions.

According to the present invention the difficulties controlling temperature and time of heating are avoided by using a continuous process instead of a batch process. The crucibles or other containers are charged onto a moving vehicle or conveyor and are moved continuously through a furnace, which may advantageously be an adaptation of the tunnel kiln used in the ceramic industry. Gases flow through the kiln in countercurrent, which permits very efficient heating, and an exact control of rate of heating and time of detention in zones of particular temperature is obtained by regulating the lengths of the zones.

25 The crucibles are preferable in fairly short rows across the car or conveyor so that very uniform heating of each crucible is possible. Because of the accurate temperature control and possibility of rapid heating without local over-heating the time required for each step in the process of forming primary ultramarine may be very drastically reduced, resulting in an important increase in output.

After the crucibles have reached the desired 35 top temperature they pass into a zone where the top temperature is maintained without increase, and remain in this soaking or detention zone the desired time. From this section they pass into the cooling zone. In this zone air is circulated 40 around the crucibles in a direction counter to their movement, absorbing heat which may be used at the other end of the tunnel to preheat the incoming crucibles. This results in a very material saving in fuel.

45 Tunnel kilns have been known for years in the ceramic industry. Their merits are well established but they are not suitable for processes which evolve corrosive or noxious gases, as is the case in the production of ultramarine where volatile sulfur compounds burn to sulfur dioxide and sulfur trioxide. This is one of the reasons why ultramarine furnace practice has not changed materially in the past eighty years. Batch furnaces built of brick or other refractory material, 50 and provided with powerful venting through the

stack which carries off combustion gases, have been considered necessary for ultramarine production. Tunnel kilns such as those used in the ceramic industry were not considered suitable, and in fact they cannot be practically used in the form in which they are normally built and operated.

We have found that by two comparatively simple modifications it is possible to use tunnel kilns with complete safety and high efficiency. It is practically impossible to design a tunnel kiln which is gas tight. We have found that it is not at all necessary to do so. A standard construction of tunnel kiln may be employed in the firing of ultramarine provided that a slight negative pressure is maintained in the kiln so that any small leaks, which are unavoidable in a practical kiln, will merely cause a slight leakage of air into the kiln. Alternatively, if in certain zones of the kiln it appears desirable to carry a pressure greater than atmospheric, then those zones are surrounded with a housing in which an air pressure slightly greater than that of the hot gases is maintained, as by a fan, for example. In one or the other of these two ways it is assured that there will be a slight leakage of air into the kiln rather than of acid gases outward.

The second modification results from the fact that the sulfur compounds in the ultramarine process burn to sulfur dioxide, and in the high temperature zones the refractory acts as a low grade catalyst so that some sulfuric acid is formed with the water vapor in the heating gases. If this acid condenses in any part of the kiln the corrosion problems are insuperable. However, we have found that by drawing off the heating gases before they reach a portion of the kiln which is at a temperature below 300° C. condensation of sulfuric acid within the kiln can be avoided and no corrosion problems result. The low temperature portion of the kiln in which the crucibles are first heated up is, of course, supplied with hot air from the cooling zone with only such boosting of temperatures by burners as may be necessary.

In the inlet zone of the kiln, in which the crucibles experience their first heating by means of hot air coming from the cooling zones, the course of travel of the heating gases is co-current with the crucible travel. Although the temperature in this zone would be low enough to permit the condensation of sulfuric acid from gas containing that substance, the co-current flow of hot air along this zone prevents the entrance of sulfuric-bearing gases from the hotter part of the kiln into this zone. The kiln is designed so that the hot air coming in co-current direction from the inlet zone meets the sulfuric-bearing gases coming countercurrent from the hot zones at the point where both of them have attained a temperature of about 300° C. At this point both types of gas are drawn off to the stack.

The temperature in the first heating zone is not high enough to cause the catalytic oxidation of any sulfur dioxide produced there to sulfur trioxide. This zone is, therefore, free from any sulfuric acid produced there, and, as explained, gas from the hot end which contains sulfuric acid cannot enter.

The present process permits a very material saving in fuel cost over the furnaces used in ultramarine plants at the present time. One reason for this is that excellent recovery of heat by heat exchange between the crucibles which are cooling and those which are heating is pos-

sible. For another thing, the usual type of ultramarine furnace stores as much or more heat in the brickwork of the furnace as in the crucibles and their contents. All this heat in the brickwork is lost during cooling and must be replaced during the next firing. By contrast, a continuous kiln, once heated, retains its heat except for the loss by radiation, etc.

Another important advantage of the present invention lies in the fact that it permits a central point for loading and unloading which makes it possible to use loading and unloading machinery, whereas in ultramarine furnaces of the standard type the crucibles have to be carefully stacked by hand. This involves considerable labor with correspondingly increased costs.

Typical operation will be described in the following examples in conjunction with the drawings in which:

Fig. 1 is a diagrammatic plan view of a tunnel kiln according to the present invention: and

Fig. 2 is a vertical section along lines 2-2 of Fig. 1.

The drawings show, in diagrammatic form, a tunnel kiln, which, in its general design, follows accepted tunnel kiln practice as used in the ceramic arts.

The kiln is shown at 1 provided with an entrance door 2 and exit door 22. A track 3 passes through the kiln on which track cars 23 travel. The cars are of conventional design provided with a solid firebrick insulating floor 24 and a superimposed hollow false floor 29 on which impervious ceramic crucibles 25 are carried in rows of four. The crucibles contain the ultramarine raw mix. In accordance with common practice for high temperature kilns, the hearth wall 26 extends nearly to the firebrick floor 24 of the car and the wheels of the car and other metal parts of the car are protected from hot gases escaping between the car floor and the kiln walls by sand seals. These consist of sand beds 27 in troughs attached to the kiln walls into which beds metal angles 28 extend downwardly from the metal framework of the cars.

The mechanism for moving the cars slowly through the kiln is conventional and is therefore not shown.

The kiln may, for example, be about 275 to 300 feet long and the speed of travel of the cars therethrough is such that it takes approximately 24 hours for a car to pass through. The kiln is shown as divided into four zones, A, B, C and D. The first, which is a preheating zone, carries the temperature of the crucibles from 15° to 300° C. The heating zone B carries the temperature from 300° to 750° C., which temperature is maintained in the firing section C and then the crucibles are cooled down to about 100° C. in section D.

In the cooling zone D cooling is effected by a circulation of cold air from the blower 4 countercurrent to the cars and crucibles moving through the zone. This air becomes heated up, for example, to about 700° C. at the hot end of zone D. At this point 5 the major portion is removed through the ducts 6 and 16 by the blowers 7 and 17, which drive the heated air through the air headers 8 and 18. The blowers 7 and 17 are adjusted so that the stream of hot air divides about evenly through the two ducts 6 and 16 and their capacity is so chosen in comparison with the capacity of the blower 4 that there exists in zone D a very slight positive pressure.

The hot air in the headers 8 and 18 is introduced into zones A and B through the pipes 14 provided with valves 20. A portion of the air

from zone D flows directly on into zone C where it is admixed with combustion gases from oil burners 13, fed from fuel headers 12 and controlled by valves 21. The hot air from the headers 8 and 18 is so adjusted that the flow of air and combustion gases through zones C and B is countercurrent to the travel of the cars carrying the crucibles but is cocurrent in zone A.

Gases and air from zones A, B and C are sucked out through the duct 9 by the exhaust fan 10 and blown into a stack 11. The exhaust is so designed that there is a slight negative pressure in zones A and B and a neutral or slightly positive pressure in zone C. This positive pressure is only sufficient to permit satisfactory operation of the burners.

At the duct 9 the temperature of the cocurrent heating air in zone A and the countercurrent flow of gases in zones B and C is above 300° C. Therefore, at this point the sulfur dioxide which is evolved in zones B, C, a part of which is transformed into sulfur trioxide by the catalytic action of the refractory lining of the kiln and united with water to form sulfuric acid, is at a temperature sufficiently high so that liquid sulfuric acid does not precipitate. As a result there is no corrosive effect on the kiln itself, the stack 11 being of suitable refractory material which is not adversely affected by sulfuric acid.

In zones A and B the pressure is negative. In zone C, however, the pressure is preferably slightly positive, and therefore this zone is surrounded with a casing 15 in which air is maintained by the blower 19 at a pressure higher than that inside the kiln. As a result any leakage will be from the atmosphere into the kiln and not the reverse, so that no hazard is encountered due to outward leakage of noxious gases.

While the rapid heating advantages of the kiln in producing primary ultramarine are enjoyed regardless of the nature of the crucibles in which the ultramarine raw mix is contained, it is preferable to use impervious ceramic crucibles so that no reactive gases encounter the raw mix during firing to primary ultramarine. The manufacture of ultramarine under conditions which prevent reactive gases from contacting the ultramarine mix is claimed in our pending application, Serial No. 606,888, filed July 24, 1945.

In the claims the term "primary ultramarine" is used in the ordinary sense, namely, to cover the product obtained in the first firing stage of the reaction before oxidation. The term "green" is no longer descriptive of the primary ultramarine, as the crude fired ultramarine of present-day production is rarely green and that of our process, never so.

We claim:

1. A continuous process for the production of "primary ultramarine" from ultramarine raw mix, which comprises: continuously moving said mix through a preheating zone and preheating

said mix to about 300° C. while said mix is moving therethrough; continuously moving the so preheated mix through a heating zone and gradually increasing the temperature of said mix to

- 5 "primary ultramarine" firing temperature while said mix is moving therethrough; continuously moving the so heated mix through a firing zone and maintaining said mix therein at said firing temperature until the formation of "primary ultramarine" is complete; continuously moving said "primary ultramarine" through a cooling zone and cooling said "primary ultramarine" gradually therein; maintaining said ultramarine mix and said "primary ultramarine" substantially out of contact with the atmospheres of all said zones but in heat-exchange relationship therewith; continuously withdrawing the atmosphere from said preheating and heating zones at a point between said zones; and causing by  
10 20 means of this withdrawal, the atmosphere in said preheating zone to flow co-currently and the atmospheres in said heating and firing zones to flow counter-currently with respect to the motion of said ultramarine mix.
- 25 2. The process according to claim 1, in which the atmospheres withdrawn from the preheating and heating zones at a point between said zones are withdrawn at a temperature of about 300° C.
- 30 3. The process according to claim 1, in which the atmospheres of at least a portion of said heating and firing zones are maintained at a slightly negative pressure with respect to the external pressures of the atmospheres surrounding said zone.

35 4. The process according to claim 1, in which at least a major portion of the heat for said preheating zone is supplied by a co-current heating gas substantially free from sulfuric acid.

- 40 5. The process according to claim 1, in which the "primary ultramarine" firing temperature is about 750° C.

WILLIAM J. KRUPPA.  
ALLING P. BEARDSLEY.  
STANLEY H. WHITING.

#### REFERENCES CITED

The following references are of record in the file of this patent:

#### UNITED STATES PATENTS

| Number       | Name    | Date          |
|--------------|---------|---------------|
| 732,264      | Boss    | June 30, 1903 |
| 1,297,629    | Wood    | Mar. 18, 1919 |
| 55 1,763,624 | Larsson | June 10, 1930 |

#### FOREIGN PATENTS

| Number   | Country       | Date          |
|----------|---------------|---------------|
| 60 9,200 | Great Britain | 1890          |
| 149,203  | Germany       | Feb. 18, 1902 |

#### OTHER REFERENCES

"Manufacture of Colors for Painting," by Riffault et al., 1874, page 305.